

## UNITED STATES PATENT OFFICE

2,203,374

PROCESS FOR THE STABILIZATION OF  
METAL ORGANIC COMPOUNDS

Johannes Andreas van Melsen, Amsterdam,  
Netherlands, assignor to Shell Development  
Company, San Francisco, Calif., a corporation  
of Delaware

No Drawing. Application November 14, 1938, Se-  
rial No. 240,337. In the Netherlands Decem-  
ber 6, 1937

12 Claims. (Cl. 44—9)

This invention relates to the stabilization of heavy metal oxy and amino methylene ketones, and more particularly is concerned with the stabilization of the iron, cobalt, nickel and copper compounds of these ketones by the addition of relatively small amounts of aromatic amines.

Oxy and amino methylene ketones may be represented by the general formula



in which  $R_1$  and  $R_2$  are hydrogen or organic radicals, such as alkyl, aryl or aralkyl radicals, and  $R_3$  is one of these organic radicals, whilst  $X$  is an 15 —OH, —NH<sub>2</sub> or —NHR<sub>4</sub> group, in which  $R_4$  represents an organic radical, such as an alkyl, aryl or aralkyl group. The organic radicals may contain substituents, preferably neutral or basic reacting, which are normally capable of forming substantially stable compounds with hydrocarbons, such as halogen, —CN, —OH, —OR, —COR, —NH<sub>2</sub>, —NHR, —NR<sub>2</sub>, —SH, —SR, —COOR, etc. Moreover,  $R_2$  and  $R_3$  together may form ring compounds.

Most of the copper and ferrous metal compounds of the above oxy and amino methylene ketones are at least partly soluble in hydrocarbon liquids and are useful as antiknock compounds for gasolines, as described in the copending application Serial No. 212,128, filed June 6, 1938, by Van Peski et al.

It has been found that under many conditions these metal ketones or their solutions in hydrocarbon liquids tend to decompose slowly, not only when exposed to light, but also in the dark. Exposure to light normally accelerates their decomposition. I have discovered that this decomposition may be greatly retarded and often substantially completely inhibited by adding to the metal ketones described above certain primary and secondary aromatic amines. Suitable amines have the formula



in which  $R_1$  is an aryl radical preferably phenyl or naphthyl radical, which may be alkylated, and which may contain preferably not more than one substitution group that is incapable of reacting under normal storage conditions with which the metal ketones to be stabilized, such as an OH, NH<sub>2</sub>, Cl, etc., group. Nitro, nitroso, acid groups, etc., attack the metal ketones and must therefore be avoided. Amines containing unsubstituted

radicals are the most effective inhibitors, and the inhibiting powers of the amines in general decrease with the number and molecular size of the substituents.  $R_2$  of the amine may be an aryl radical of the same type as  $R_1$ , or hydrogen, 5 or a relatively small aliphatic or naphthenic radical having preferably not more than eighteen carbon atoms. Particularly effective amines are aniline and diphenyl amine. Other highly active amines are toluidine, methyl aniline, naphthyl 10 amine. Somewhat less effective are for example the amino phenols, phenylene diamines, chloroanilines, etc. The amounts of inhibitor required to effect stabilization are normally quite small, usually less than an equal weight of the metal 15 ketone, although larger amounts may be used if desired. In many instances substantially complete stabilization was achieved with 5 to 10% by weight of the inhibitor.

In addition to the inhibitors, other substances 20 may be added such as mutual solvents or diluents. For example, a small amount of benzene frequently improves the homogeneity of non-homogeneous mixtures of the metal ketones and the herein described inhibitors, thereby improving 25 the stabilizing effect of the inhibitor. If mutual solvents are required to improve homogeneity, I prefer to use amounts of the solvents at least sufficient to insure complete miscibility at about room temperature. The amounts of mutual sol- 30 vents required to produce this result naturally will vary within extremely wide limits, i. e., from nothing or a bare trace to several times the volume of the mixture, and must be determined experimentally for different mixtures. Aside from 35 benzene, other suitable mutual solvents are for instance lower alcohols, ethers, ketones, aliphatic amines, aromatic normally liquid hydrocarbons in general, etc. Furthermore metal ketones suitable as anti-knock agents may be dissolved in 40 gasoline type fuels which themselves are substantially stable, such as straight-run, cracked or polymer gasolines, branched chain lower ethers, ketones, alcohols, etc., and solutions so produced may be stabilized by the addition of suitable 45 amounts of my inhibitors. Thus antiknock fuels ready for use in spark ignition engines, or concentrates of such fuels to be used for blending, containing effective amounts of the metal-ketone antiknock agents may be produced, which are 50 stable in storage for periods of many months, and which in the absence of the inhibitor might deteriorate.

While, in the foregoing, I have stressed in particular the stabilization of the ketone compounds 55

of the ferrous metals and copper because of the importance of these compounds as antiknock agents in gasoline type fuels, it shall be understood that corresponding compounds of other heavy metals which are capable of uniting with the ketones herein described to form relatively stable compounds, may be stabilized equally well.

The following examples further illustrate my invention.

10 *Example I*

15 A sample of the liquid copper compound of ethyl amino methylene acetone decomposed, when standing in semi-darkness for two weeks in a closed glass bottle, to the extent of settling out a small amount of a solid substance. Another sample of the same compound containing 10% by weight aniline, stored under identical conditions showed no sign of decomposition after 20 two months.

20 A third sample containing 10% by weight diphenyl amine also was completely undecomposed after two months standing under the above conditions.

25 *Example II*

30 To the cobalt compound of ethyl amino methylene acetone an equal weight of aniline was added. The mixture was exposed to light for 10 days and remained clear. In the absence of 35 aniline the cobalt compound decomposed considerably under the above conditions, forming a precipitate.

I claim as my invention:

35 1. The process of stabilizing a compound selected from the class consisting of copper and ferrous compounds of oxy and of amino methylene ketones comprising adding to said compound an aromatic amine



40 in which  $\text{R}_1$  is phenyl and  $\text{R}_2$  is a radical selected from the group consisting of hydrogen and phenyl.

45 2. The process of stabilizing a compound selected from the class consisting of copper and ferrous compounds of oxy and of amino methylene ketones, comprising adding to said compound an aromatic amine



50 in which  $\text{R}_1$  is phenyl and  $\text{R}_2$  is a radical selected from the group consisting of hydrogen and phenyl, and further adding an amount of a mutual solvent for said compound, said amount being sufficient to produce a homogeneous mixture.

55 3. A composition of matter comprising a compound selected from the class consisting of copper and ferrous compounds of oxy and of amino methylene ketones, in admixture with an aromatic amine



60 65 in which  $\text{R}_1$  is phenyl and  $\text{R}_2$  is a radical selected from the group consisting of hydrogen and phenyl.

4. The composition of claim 3 containing an

amine, in which at least one of the radicals  $\text{R}_1$  and  $\text{R}_2$  is an unsubstituted aryl radical.

5. The composition of claim 3 containing an amine, in which at least one of the radicals  $\text{R}_1$  and  $\text{R}_2$  is a phenyl radical.

6. The composition of claim 3 in which the amine is aniline.

7. The composition of claim 3 in which the amine is diphenyl amine.

8. The composition of claim 3 in which the amount of the amine is from 5 to 100% by weight of the metal compound.

9. A composition of matter comprising a compound selected from the class consisting of copper and ferrous compounds of oxy and of amino methylene ketones, in admixture with an aromatic amine



20 in which  $\text{R}_1$  is phenyl and  $\text{R}_2$  is a radical selected from the group consisting of hydrogen and phenyl, and with a mutual solvent for said compound and amine.

25 10. A homogeneous composition of matter comprising a compound selected from the class consisting of copper and ferrous compounds of oxy and of amino methylene ketones, in admixture with an aromatic amine



30 in which  $\text{R}_1$  is phenyl and  $\text{R}_2$  is a radical selected from the group consisting of hydrogen, and phenyl, and with a mutual solvent for said compound and amine in an amount at least sufficient to insure complete miscibility of the components at normal room temperature.

35 11. A gasoline type antiknock motor fuel of improved stability for spark ignition engines comprising a substantially stable gasoline type 40 motor fuel, an effective amount of an antiknock agent selected from the class consisting of copper and ferrous compounds of oxy and of amino methylene ketones in admixture with an aromatic amine



45 in which  $\text{R}_1$  is phenyl and  $\text{R}_2$  is a radical selected from the group consisting of hydrogen and phenyl.

50 12. A homogeneous composition of matter comprising a compound selected from the class consisting of copper and ferrous compounds of oxy and of amino methylene ketones, in admixture with an aromatic amine



55 of which  $\text{R}_1$  is phenyl and  $\text{R}_2$  is a radical selected from the group consisting of hydrogen and phenyl and with a mutual solvent for said compound and amine in an amount at least sufficient to insure complete miscibility of the components at normal room temperature, the amount of said amine being from 5 to 100% by weight of the metal compound.

JOHANNES ANDREAS VAN MELSEN.